



US005598633A

**United States Patent**

[19]

**Hartz**[11] **Patent Number:** **5,598,633**[45] **Date of Patent:** **Feb. 4, 1997**[54] **METHOD OF MANUFACTURING A CASTER ROLL CORE AND SHELL ASSEMBLY**[75] Inventor: **Warren C. Hartz**, McKenzie, Tenn.[73] Assignee: **Norandal USA, Inc.**, Brentwood, Tenn.[21] Appl. No.: **392,427**[22] Filed: **Feb. 22, 1995****Related U.S. Application Data**

[63] Continuation-in-part of Ser. No. 274,186, Jul. 12, 1994.

[51] **Int. Cl.<sup>6</sup>** ..... **B23P 15/00**[52] **U.S. Cl.** ..... **29/895.212; 29/895.32; 492/46**[58] **Field of Search** ..... **29/895.2, 895.212, 29/895.32; 492/46, 54, 33, 35, 1, 3; 164/442, 444, 448; 165/89, 90**

[56]

**References Cited****U.S. PATENT DOCUMENTS**

|           |         |                      |            |
|-----------|---------|----------------------|------------|
| 4,071,081 | 1/1978  | Chielens et al. .... | 165/90     |
| 4,773,468 | 9/1988  | Lauener ....         | 492/46     |
| 5,209,283 | 5/1993  | Miltzow et al. ....  | 164/448    |
| 5,265,332 | 11/1993 | Hartz ....           | 29/895.212 |
| 5,292,298 | 3/1994  | Scannell ....        | 492/46     |

*Primary Examiner*—Irene Cuda  
*Attorney, Agent, or Firm*—Keck, Mahin & Cate

[57] **ABSTRACT**

An improved caster roll core and shell assembly are manufactured wherein two overlays of stainless steel of different hardness are deposited on the surface of the roll core, thus prolonging the life of the roll.

**7 Claims, 2 Drawing Sheets**

FIG. 1A



FIG. 1B



## METHOD OF MANUFACTURING A CASTER ROLL CORE AND SHELL ASSEMBLY

This application is a continuation in part of Ser. No. 10  
08/274,186 filed Jul. 12, 1994, now abandoned.

### FIELD OF THE INVENTION

The present invention is concerned with an improved 10  
caster roll core and shell assembly wherein a chromium  
layer is plated onto the inside surface of the shell and two  
overlays of stainless steel of different hardness are deposited  
on the surface of the roll core, thus significantly prolonging  
the life of the roll.

### BACKGROUND OF THE INVENTION

In the manufacture of aluminum foils or sheets, conventional 20  
twin roll continuous sheet casting machines comprise a pair of parallel, water-cooled, counter-rotating rolls. After  
being in use for a given period, the surface of the roll must be reground because of heat cracks resulting from thermal  
fatigue and out-of-roundness due to galling between caster  
core and shell. Accordingly, the shells surrounding the cores  
must be removed periodically, and the cores repaired and  
reground before rebuilding of the roll assembly.

The major cause of damage to caster roll assemblies is 25  
galling between the core and the shell, which occurs when  
the shell slips relative to the core under load. Cold welding  
of the core and shell during relative motion causes metal to  
be torn from the core and displaced in the interface between  
the two, resulting in distortion of the rolls and roll gap,  
creating bad shape in the continuously cast sheet.

Using such conventional roll assemblies, it is possible to 30  
cast from about 10 to 12 millions pounds of aluminum sheet  
before cutting of the shells and repairing and regrounding the  
cores. However, after regrounding two or three times, the  
hardened layer on the core surface is lost and the cores are  
destroyed by deformation. To overcome this problem, it  
became general practice to coat cores with a stainless steel  
overlay. This modification extended the service life between  
regrounding by about 50% and avoided destruction of cores  
by weld rebuilding to original dimensions and regrounding.  
However, the stainless steel weld overlay is still subject to  
cold welding and galling between the shell and the core.

Another approach to extend the service life of the core is 35  
to coat the inner surface of the shell with hard chromium, as  
proposed in U.S. Pat. No. 5,265,332, which is hereby  
incorporated by reference. Again, however, usual problems  
with the stainless steel overlay are present.

There is therefore a great need to develop a core having 40  
an extended service life between shell removal. Preferably,  
the core would be prepared by simple techniques at a  
reasonable cost.

### SUMMARY OF THE INVENTION

In accordance with the present invention, there is now 45  
provided an improved caster roll core and shell assembly  
wherein the surface of the core is coated with two overlays  
of stainless steel, each having a distinct hardness. In the  
preferred embodiment of the invention, the overlay of stain-  
less laying on the surface of the core is softer than the  
external overlay of stainless steel.

The present invention also comprises the method for  
manufacturing the improved core.

### IN THE DRAWINGS

FIG. 1 is a perspective view of the core of a roll according  
to the present invention.

### DETAILED DESCRIPTION OF THE INVENTION

The present application discloses a roll and shell assembly 10  
for making metal sheets, preferably aluminum, wherein the  
core of the roll comprises a dual layer stainless steel overlay  
which shows significantly improved properties over the rolls  
currently known. When used in combination with shells  
having the inner surface coated with chromium, the service  
life between shell removal and rebuilding of the rolls is  
extended by as much as 400%. Furthermore, the cores are  
found to be relatively undamaged.

Referring to FIGS. 1A and 1B which illustrates a preferred 15  
embodiment of the present invention, there is found a roll 10 comprising a core 12 having a plurality of water  
channels 13 for cooling, the core 12 being coated with an  
overlay of stainless steel 14. The thickness of this one pass  
overlay is preferably at least  $\frac{1}{8}$ , and preferably has a  
hardness of from 20 to 25 on the Rockwell "C" scale. An example of a suitable stainless steel 14 is LINCORE 30,  
manufactured and sold by Lincoln Electric, Cleveland,  
Ohio. It should be noted that overlay 14 may be formed by  
welding several layers of  $\frac{1}{8}$ " each until the desired thickness  
is reached.

Onto overlay 14 is laid another overlay of stainless steel 20  
16 having a thickness of at least  $\frac{1}{8}$ ", preferably less than 1",  
and most preferably  $\frac{5}{8}$ ", and a hardness of from 50 to 56 on  
the Rockwell "C" scale. An example of a suitable stainless  
steel 16 is LINCORE 96S, manufactured and sold by  
Lincoln Electric, Cleveland, Ohio. Overlay 16 is preferably  
formed by welding several layers of about  $\frac{1}{8}$ " each until the  
desired thickness is reached. This provides a structure having  
better mechanical properties and increased resistance to  
wear and tear. Once core 12 is coated with overlays 14 and  
16, water channels 13 are cut therein. This operation can be  
carried out with any conventional router, and is rendered  
necessary to insure that shell 18 (discussed below) is properly  
cooled when the roll is in use.

A further advantage of overlays 14 and 16 is that they 25  
substantially eliminated the breaking of the sidewalls of the  
water channels in the core, which took place when the core  
was not provided with these overlays.

Finally, shell 18 preferably made of alloy steel having its 30  
inner surface coated with a layer of chromium having a  
thickness of from 0.001 to 0.01 inch in the manner described  
in U.S. Pat. No. 5,265,332, is shrink-fitted around overlay 16  
in a conventional manner. It is believed that overlay 14 acts  
as an interface or cushion between the core and overlay 16  
to prevent cracking and separation of the two when under  
stress.

In operation, the molten metal is passed between two 35  
rolls, cooled, and ejected as a metal sheet. The thickness of  
the sheet is adjusted by varying the space between the rolls.  
The present roll and shell assembly is particularly useful for  
manufacturing aluminum sheets, but sheets of other metals  
like copper, zinc and the like, may also be manufactured  
with these roll and shell assemblies.

The method for obtaining a roll 10 can be described as 40  
65 follows. A core 12 made of conventional material, for  
example steel or alloyed steel, is installed in a chamber and  
heated to a temperature of from 200° to 275° C. until the

core is hot through the entirety of its structure (4-5 hours). Preferably, before heating the rolls, graphite plugs have been inserted in the holes of the channels in the core. Then, a first layer of stainless steel is welded onto the core, and this operation is repeated until the desired thickness of overlay 5

14 is reached. Subsequently, a first layer of stainless steel having a hardness higher than that of overlay 14 is welded on overlay 14, and this operation is repeated until the desired thickness of overlay 16 is obtained. The roll is then placed in an insulated box and heated to a temperature of from 200° to 275° C. The box is closed and the temperature is maintained to 200°-275° C. for another 6-8 hours. The temperature is then lowered slowly to room temperature. It should be noted that during all the above process, the roll is preferably turning at a speed of about 1 rpm. Finally, the water channels 10

15 13 are cut in overlays 14 and 16. While the invention has been described in connection with specific embodiments thereof, it will be understood that it is capable of further modifications and this application is intended to cover any variations, uses or adaptations of the invention following, in general, the principles of the invention and including such departures from the present disclosure as come within known or customary practice within the art to which the invention pertains, and as may be applied to the essential features hereinbefore set forth, and as follows in the scope of the appended claims.

What is claimed is:

1. A method for manufacturing a roll for making metal sheets or foils, the roll comprising:  
a core having a plurality of cooling channels;  
a first overlay of stainless steel on the core; and

a second overlay of stainless steel on the first overlay of stainless steel, the second overlay having a hardness higher than the hardness of the first overlay, the method comprising the steps of:

heating the core to at least 200° C.;  
welding the first overlay on the core;  
welding the second overlay on the first overlay;  
maintaining the temperature to at least 200° C. for several hours;  
cooling the core to room temperature;  
cutting the cooling channels in the first and second overlays and  
shrink-fitting a shell onto the core.

2. A method according to claim 1, wherein the hardness of the first overlay is from 20 to 25 on the Rockwell "C" scale, and the hardness of the second overlay is from 50 to 56 on the Rockwell "C" scale.

20 3. A method according to claim 1, wherein the thickness of the first overlay of stainless steel is lower than the thickness of the second overlay of stainless steel.

4. A method according to claim 1, wherein the thickness of the first overlay is about  $\frac{1}{8}$ ", and the thickness of the second overlay is at least  $\frac{1}{8}$ ".

5. A method according to claim 1, wherein the first and second overlays are made of several layers.

6. A method according to claim 1, wherein the shell has its inner surface electroplated with chromium.

25 30 7. A method according to claim 1, wherein the metal is aluminum.

\* \* \* \* \*